# EUROPEAN PATENT APPLICATION

(11) **EP 1 724 327 A1**
(43) Date of publication of application: **22.11.2006**
(21) Application number: 05710999.3
(22) Date of filing: 18.01.2005
(51) Int. Cl.: C10L 1/32

(54) **FUEL PRODUCTION METHOD (VARIANTS)**

(30) Priority: 24.02.2004 RU 2004105114
(71) Applicant: Zhirnokleev, Igor Anatolievich, Moscow, 109052 (RU); Sidorov, Viktor Viktorovich, Moscow, 127322 (RU)
(72) Inventor: Zhirnokleev, Igor Anatolievich, Moscow, 109052 (RU); Sidorov, Viktor Viktorovich, Moscow, 127322 (RU)
(74) Representative: Einsel, Martin
(86) International application number: PCT/RU2005/000014
(87) International publication number: WO 2005/080534

(57) **Abstract**

This invention relates to production of water-fuel emulsions to be used for various purposes from industrial wastes, oil residues, hydrocarbon components, and water-containing components (fuel oil-containing water, waste lubricating coolants, and so on), and can be used for processing and utilizing wastes of liquid and thickened hydrocarbons (oil, fuel oil, vegetable and mineral oils, oil slimes, fuel oil slimes, paraffins, asphaltenes, and so on). This method of producing fuel from oil residues and a hydrocarbon component comprises heating them, cleaning them from mechanical impurities, and mixing them in a turbulent flow until the hydrocarbon component is distributed in the oil residue mass at a homogeneity factor of less than 0.5. The mixing temperatures of oil residue and hydrocarbon component differ by 10°C or less. The mixing product is then homogenized in a mechanical rotary disperser until the maximum size of dispersed phase particles is 50 microns or less, for an average size of 1 to 15 microns. Water or a water-containing component is then added to the homogenized mixture mass in a turbulent flow to obtain its distribution in the mixture mass at a homogeneity factor of at least 0.5, the temperatures of the streams differing by 10°C or less, and homogenization in the mechanical rotor disperser continues until the maximum size of water particles in ready fuel is 50 microns or less, for an average size of 1 to 15 microns. The total water content in the fuel may vary within the range of 5% to 60% by weight. Fuel oil-containing water, fuel-containing discharges, waste lubricating coolants, or process water may be used as water. The specification also discloses a method of producing fuel from distillate fractions boiling away at a temperature of 180°C or above by heating them, cleaning them from mechanical impurities, stirring, and homogenizing them in a turbulent flow, in which a component containing water and a surfactant is added to the homogenized mixture mass in a turbulent flow until water is distributed in the mixture mass at a homogeneity factor of at least 0.5, the temperatures of the streams differing by 100°C or less, whereupon the mixture is homogenized in a mechanical rotor disperser until the maximum size of water particles in ready fuel is 50 microns or less, for an average size of 1 to 10 microns. Waste lubricating coolant is used as the component containing water and a surfactant.

## Description

### FIELD OF THE INVENTION

This invention relates to production of water-fuel emulsions to be used for various purposes, using industrial wastes, oil residues, hydrocarbon components, and water-containing components (fuel oil-containing water, lubricating coolants, and so on), and can be used for processing and utilizing wastes of liquid and thickened hydrocarbons (oil, fuel oil, diesel fuel, vegetable and mineral oils, oil slime, fuel oil slime, paraffins, asphaltenes, and so on).

### BACKGROUND OF THE INVENTION

A known prior art method is used to produce water-fuel emulsions by processing and utilizing hydrocarbon wastes by heating the wastes, adding water thereto, mixing the wastes with a heavy liquid fuel, dispersing the resulting mixture to obtain a water-fuel emulsion, and delivering the water-fuel emulsion to a burner. The hydrocarbon wastes are heated to a temperature of 20°C to 90°C, with or without water added, the hydrocarbon wastes are mixed with fuel, and the resulting mixture is dispersed simultaneously in a pulsating-rotor homogenizing mixer at a working clearance of 50 to 250 microns and shear rate of at least 10 m/sec, the hydrocarbon wastes and fuel being fed into the homogenizing mixer at a ratio of 1:15 to 1:1.5.

The homogenizing process is monitored using a measuring microscope according to water-fuel emulsion samples, or visually by the appearance of the flame, with dispersed phase particles in water-fuel emulsion exceeding 10 microns, or decreasing brightness and transparency of the flame, and when traces of soot are detected in the flame tail the revolutions of the homogenizing mixer motor are increased, or a portion of the water-fuel mixture is recycled from the homogenizing mixer outlet to the inlet thereof, or the flow rate of fuel entering the homogenizing mixer is raised, or the flow rate of hydrocarbon wastes at the inlet of the homogenizing mixer is reduced (RU 2,204,761, May 20,2003).

A drawback of the prior art method is that the target products contain a significant proportion of undesired impurities that have a disadvantageous effect on the quality of the products.

In another prior art method, fuel is produced by mixing waste lubricating oil and water or a water-containing component and oil residue, and homogenizing the mixture, in which case the waste oils are subjected to preliminary mechanical treatment (RU 2,150,489, June 10, 2000, C10L 1/32).

A further prior art method is used to produce fuel from a mixture of oil residues and hydrocarbon components by heating them, cleaning them from mechanical impurities, and mixing them in a turbulent flow (PL 131,427, C10L 1/04, December 30, 1985).

This prior art method is not intended to produce fuels with a high water content that are highly resistant to separation.

In still another prior art method, fuels are produced by mixing distillate fractions boiling away at above 180°C and water (up to 20%), followed by homogenizing them in a turbulent flow in a rotary impact mill (US 4;394,131, C10L 1/32, July 19, 1983).

### DISCLOSURE OF THE INVENTION

It is an object of this invention to produce fuels with a high water content (up to 70%) at a high dispersion rate, which possess a high stability.

This object is achieved by a method of producing fuel from oil residues and a hydrocarbon component by heating them, cleaning them from mechanical impurities, and then mixing them in a turbulent flow to cause the hydrocarbon component to be dispersed in the oil residue mass at a homogeneity factor of at least 0.5. Moreover, the temperatures at which the oil residue and the hydrocarbon component are mixed differ by 10°C or less. The mixing product is then homogenized in a mechanical rotor disperser to achieve a maximum dispersed phase particle size of, or under, 50 microns, for an average particle size of 1 to 15 microns, followed by adding water or a water-containing component to the homogenized mixture in a turbulent flow to achieve a homogeneity factor thereof in the mixture mass of at least 0.5, temperatures of the feedstock streams differing by 10°C or less, and homogenizing the components preferably in a mechanical rotor disperser to achieve a maximum water particle size of 50 microns or less in ready fuel, for an average size of 1 to 15 microns.

It is preferred to control the viscosity of the resulting fuel at the first stage where the oil residue and hydrocarbon component are mixed and at the second stage where water is added.

Water can alternatively be replaced with fuel oil-containing water, fuel-containing discharges, waste lubricating coolants, process water, and so on.

When water-containing fuel oil having over 2% by weight of water is used, it is preferred to subject it to coarse homogenization in a turbulent flow to obtain an average water particle size of 50 to 100 microns, to be followed by dispersion thereof to an average water particle size of 1 to 15 microns.

Oil residues can alternatively be replaced with fuel oil grades M-40, M-100, F-5 and F-12, long-storage fuel oils, waste petroleum products, and so on.

Hydrocarbon components can include low-grade diesel fuel, kerosene, heavy gasoline, and so on.

In another embodiment of this method of producing fuel, distillate fractions boiling away at or above 180°C, which are used for producing fuel, are heated, cleaned from mechanical impurities, a water-containing component is added thereto, mixing and homogenizing them in a turbulent flow, wherein the water-containing component is a component further containing a surfactant, and the mixture is stirred to achieve dispersion of water in the mixture mass at a homogeneity factor of at least 0.5 and at the temperatures of the component streams differing by or under 10°C, followed by homogenizing the mixture, preferably in a mechanical rotor disperser to achieve a maximum water particle size of or below 50 microns, for an average size of 1 to 10 microns, in ready fuel.

It is preferred to use waste lubricating coolant as a component containing water and a surfactant.

It is preferred, in both embodiments, to maintain the total water content in ready fuel within the range of 5% to 60% by weight, and it is also preferred to heat the fuel component streams to a temperature of 40°C to 120°C.

### PREFERRED EMBODIMENTS OF THE INVENTION

The method of this invention is performed as follows:

Oil residues, waste petroleum products, hydrocarbon components, water or water-containing components are subjected separately to preliminary treatment, including heating the components to a desired temperature (40°C to 120°C), with the temperatures of the streams differing by 10°C or less, and filtering off mechanical impurities. The resulting oil residues, hydrocarbon component, and, if necessary, waste petroleum products of desired quality are taken in desired quantities and delivered to a feed mixture preparation station to be mixed thereafter in a turbulent flow to cause the hydrocarbon component to be distributed in the oil residue mass at a homogeneity factor of at least 0.5 (preferably at least 0.85). The temperatures at which the oil residue and hydrocarbon component are mixed differ by 10°C or less. The mixture is then homogenized in a mechanical rotor disperser to achieve a maximum dispersed phase particle size of or under 50 microns, for an average particle size of 1 to 15 microns (preferably 3 to 10 microns).

The homogenized mixture prepared at this stage and heated water or a water-containing component are fed to the mixing and homogenizing station where they are distributed in the mixture mass in a turbulent flow at a homogeneity factor of at least 0.5 (preferably at least 0.85) and at the temperatures of the streams differing by 10°C or less, and homogenized in a mechanical rotor disperser to obtain a maximum size of water particles of or under 50 microns in ready fuel, for an average size of 1 to 15 microns (preferably 3 to 10 microns).

The result is a composite water-fuel oil fuel, or water-fuel oil mixture, when water-containing products are added to oil residues, suitable for use as, for example, boiler, furnace, ship and other fuels.

In the second embodiment of the method of producing fuel, distillate fractions boiling away at a temperature of 180°C or above are heated to a temperature of 40°C to 120°C, cleaned from mechanical impurities, a water-containing component also containing surfactants, such as waste lubricating coolants, being added thereafter, stirred and homogenized in a turbulent flow, stirring being continued until water is distributed in the mixture mass at a homogeneity factor of at least 0.5 (preferably at least 0.85), at temperatures of the streams differing by 10°C or less, and homogenized in a mechanical rotor disperser to obtain a maximum size of water particles of or under 50 microns in ready fuel, for an average size of 1 to 10 microns (preferably 3 to 6 microns). The result is a boiler fuel based on distillate fractions.

The method is illustrated by the following examples:

### Example 1

Fuel oil grade M-40, waste mineral oil, low-grade diesel fuel, and process water used in this example are each heated, strained, and dosed. Fuel oil, waste oil, and diesel fuel strained to remove mechanical impurities and heated to a temperature of about 90°C (±5°C) are fed at a ratio of 1:1:1 by mass to a feedstock mixture preparation station, where they are stirred in a turbulent flow to obtain waste oil distribution in the fuel oil mass at a homogeneity factor of 0.92, and homogenized in a mechanical rotor disperser to obtain a maximum size of dispersed phase particles of 30 microns, for an average size of 3 to 10 microns. The resulting homogeneous mixture is then fed to a mixing and homogenizing station that is also supplied with lubricating coolant subjected to preliminary treatment (heated to 90°C and strained) at a rate of 40% by weight. Also at this station, the mixture is homogenized in a mechanical rotor disperser to give a maximum water particle size of 30 microns in ready fuel, for an average particle size of 3 to 10 microns and a homogeneity factor of 0.92.

The result is a highly dispersed composite water-fuel oil fuel possessing a high resistance to separation in long storage (at least 30 days).

### Example 2

Water-containing fuel oil, with 10% by weight of water, is subjected to coarse homogenization in a turbulent flow in a pipeline to an average water particle size of 75 microns. Heavy diesel fuel is used as a hydrocarbon component, and fuel oil-containing water is used as water. The process is then conducted as in Example 1, except that the homogeneity factor of diesel fuel in fuel oil is 0.9 and all the components are heated to a temperature of approximately 100°C (±5°C). The quantity of water added to the last-in-line mixing and homogenizing station is 30% by weight, and the emulsion is obtained at a water homogeneity factor of 0.9. The result is a highly dispersed water-fuel oil fuel having a high resistance to separation in long storage (50 days).

### Example 3

Each of fuel oil grade M-100 and heavy gasoline used in this example are separately heated, strained, and dosed. Strained from mechanical impurities and heated to a temperature of approximately 50°C (±5°C) at a ratio of 1:2, the fuel oil and heavy gasoline are fed to a feedstock mixture preparation station, where they are mixed in a turbulent flow until gasoline is distributed in the fuel oil mass at a homogeneity factor of 0.95 and homogenized in a mechanical rotor disperser to obtain a maximum size of dispersed phase particles of 30 microns, for an average size of 3 to 10 microns. The resulting homogenized mixture is then fed to a mixing and homogenizing station, which is also supplied with water following preliminary treatment (heated to 50°C and filtered) at a rate of 50% by weight. The mixture is homogenized in the mechanical rotor disperser at this station to a maximum size of water particles of 30 microns in ready fuel, for an average size of 3 to 10 microns and a homogeneity factor of 0.95. The result is a highly dispersed water-fuel oil mixture having a high resistance to separation in long storage (50 days).

### Example 4

A distillate fraction boiling away in the temperature range of 180°C to 350°C and a surfactant-containing lubricating coolant are heated separately to a temperature of 85°C and cleaned from mechanical impurities. Waste lubricating coolant is then added to the hydrocarbon fraction, stirred and homogenized in a turbulent flow, stirring being continued until water is distributed in the mixture mass at a homogeneity factor of 0.87 and at temperatures of the streams differing by 10°C or less, followed by homogenization in a mechanical rotor disperser to obtain a maximum size of water particles of or under 30 microns in ready fuel, for an average particle size of 3 to 6 microns. The result is a highly dispersed boiler fuel having a high resistance to separation in long storage (90 days).

This invention is, therefore, suitable for making high-quality products from inexpensive feedstock.

## Claims

1. A method of producing fuel from oil residues and a hydrocarbon component by heating, straining them to remove mechanical impurities, and mixing them in a turbulent flow, wherein mixing is continued until the hydrocarbon component is distributed in the oil residue mass at a homogeneity factor of at least 0.5 at temperatures of the oil residue and hydrocarbon component mixed differing by 10°C or less, followed by homogenizing the mixing product in a mechanical rotor disperser to obtain a maximum size of dispersed phase particles of or under 50 microns, for an average size of 1 to 15 microns, adding water or a water-containing component to the homogenized mixture mass in a turbulent flow until the water particles are distributed in the mixture mass at a homogeneity factor of at least 0.5 and at temperatures of the streams differing by 100°C or less, and homogenizing the mixture until the maximum size of water particles in ready fuel is 50 microns or less, for an average size of 1 to 15 microns.

2. A method as set forth in claim 1, wherein the viscosity of the fuel produced is controlled at the first stage by mixing the oil residue and hydrocarbon component, and at the second stage, by adding water.

3. A method as set forth in claim 1, wherein waste petroleum products, low-grade diesel fuel, kerosene or heavy gasoline are used as the hydrocarbon component.

4. A method as set forth in claims 1 and 2, wherein fuel oil-containing water, fuel-containing discharges, waste lubricating coolants, and process water are used as water or the water-containing component.

5. A method as set forth in claim 1, wherein water-containing fuel oil having over 2% by weight of water, which is used as oil residue, is subjected to coarse homogenization in a turbulent flow in a pipeline until the average size of water particles reaches 50 to 100 microns and then dispersed to obtain an average size of water particles in the range of 1 to 15 microns.

6. A method as set forth in claim 1, wherein the total content of water in ready fuel is maintained in the range of 5% to 60% by weight.

7. A method as set forth in claim 1, wherein the streams of fuel components are heated to a temperature of 40°C to 120°C.

8. A method of producing fuel from distillate fractions boiling away at a temperature of or above 180°C by adding a water-containing component, mixing, and homogenizing them in a turbulent flow, wherein the distillate fractions and the water-containing component are heated separately and cleaned from mechanical impurities, the water-containing component being a component further containing a surfactant, and stirring is continued until water is distributed in the mixture mass at a homogeneity factor of at least 0.5 at temperatures of the streams differing by 10°C or less, and homogenizing the mixture until the maximum size of water particles in ready fuel is 50 microns or less, for an average size of 1 to 10 microns.

9. A method as set forth in claim 8, wherein waste lubricating coolant is used as a component containing water and a surfactant.

10. A method as set forth in claim 8, wherein the total water content in ready fuel is in the range of 5% to 60% by weight.

11. A method as set forth in claim 8, wherein the streams of fuel components are heated to a temperature in the range of 40°C to 120°C.
